

Aug. 4, 1931.

H. D. RICE

1,817,323

PROCESS OF MAKING RUBBERIZED SHEET MATERIALS AND PRODUCTS

Filed March 22, 1929

*Fig. 1.*



*Fig. 2.*



*Fig. 3.*



*Fig. 4.*



*Fig. 5.*



BY

Harold D. Rice *INVENTOR*  
Ernest Hopkinson *ATTORNEY*

## UNITED STATES PATENT OFFICE

HAROLD D. RICE, OF BRISTOL, RHODE ISLAND, ASSIGNOR TO WOONSOCKET RUBBER COMPANY, OF MILLVILLE, MASSACHUSETTS, A CORPORATION OF RHODE ISLAND

## PROCESS OF MAKING RUBBERIZED SHEET MATERIALS AND PRODUCTS

Application filed March 22, 1929. Serial No. 349,071.

This invention relates to a process for making rubberized sheet material, more particularly to a sheet material having the characteristics of finished leather, and to the product.

There are a number of substitute or imitation leathers on the market in which a fabric base is provided with a nitro-cellulose or similar coating treated to simulate various leather effects. These products are relatively expensive to make by reason of the use of a cloth backing, and by reason of the number of spreading and other operations required to apply and properly finish a nitro-cellulose coating of the required thickness. In addition, materials of this character depend almost wholly for their strength on the cloth backing. Furthermore, unless the edges of the cloth backing are treated in some manner they tend to fray in a comparatively short time, giving a ragged edge.

An object of the present invention is to provide a method for making a rubberized sheet material which is cheap, durable, flexible, waterproof throughout, having a relatively high tensile strength, giving an edge which when cut resembles that of leather, having no tendency to fray, and which can be given various finishes to simulate different leathers. The invention also comprises the article.

The invention broadly consists in hardening relatively cheap fibres into a bat, impregnating the bat with rubber in fluid form, compacting the bat, coating it with rubber, and where embossing is desired first superficially treating the coating with a halogen and then embossing, vulcanizing and finishing the material by a surface halogenating treatment.

For a complete disclosure of the nature and objects of the invention, reference is had to the accompanying specification and drawings, in which latter:

Fig. 1 is a perspective of a piece of completed hardened bat of fibre;

Fig. 2 is a similar view showing the piece after impregnation with rubber and partial consolidation;

Fig. 3 is a similar view of the piece as reduced to its final thickness by pressing;

Fig. 4 is a perspective of a piece of the finished sheet material; and

Fig. 5 is a diagrammatic view of a suitable apparatus for impregnating the bat.

In carrying out the invention, a bat of fibres is first formed, preferably by blending fibres of rayon, hemp, wool and cotton in a blender and picker, the blend then being made up into a bat on a cross forming carding machine; superimposing one thin layer on top of another, with the fibres in one layer running at right angles to those in an adjoining layer, until the desired weight is attained. A suitable blend of fibres is rayon 50 parts, wool 10 parts, cotton 20 parts, and hemp 20 parts. While the invention is not limited to the specific amounts given or to the specific kind of fibres named, the above-described blend has been found very suitable. The rayon is valuable by reason of its long fibre, its cleanliness and low cost. The hemp also has a low cost and imparts strength. The wool is valuable for its hardening characteristics; and the cotton is used as a filler. While a straight forming carding machine can be used, it is preferred to use a cross forming carder, since it gives a stronger bat with greater resistance to tearing and separation after impregnation. If desired to obtain still greater strength, a woven cotton web, such as an open sheeting may be introduced near the middle of the bat, between two layers of the carded material.

The bat is then subjected to a process known in the art as "hardening", which imparts sufficient strength for succeeding operations. In this operation the bat is wet with water, folded up on itself, and operated on by hammers which act to compact the fibers to some extent without, however, felting them together in the sense that the term "felting" is ordinarily employed. The moist bat is then unfolded and is ready to be impregnated with rubber.

The bat 1 thus produced is relatively loose and thick, and has the general appearance as shown in Fig. 1. While the bat may be dried and impregnated with rubber in the

form of cement, it is preferred to operate directly on the moist bat and impregnate it with a water dispersion of rubber, such as natural or artificial latex.

5 In Fig. 5 there is shown a suitable form of impregnating apparatus, in which the bat 1 is drawn over a guide roll 2, before entering the latex bath 3. The bat then passes underneath a roll 4 partly submerged in the latex 10 and passes from this roll beneath a second roll 5, and then between the rolls 5 and 6, and finally between the rolls 6 and 7. During its passage through the bath the bat becomes thoroughly impregnated with the latex and 15 any excess is squeezed out by the rolls 5, 6 and 7, which also partly consolidate the bat. The top roll 7 preferably has a rubber surface, while the other rolls may be of metal.

If natural latex is used, it is preferred to 20 employ a latex which has been subjected to one of the well-known creaming processes, by which the water solubles present in the latex are greatly reduced and the latex concentrated. However, normal latex, vulcanized latex or any suitable artificial dispersion 25 of rubber may be used. A suitable latex compound is as follows:

|                                                                                                          | Parts |
|----------------------------------------------------------------------------------------------------------|-------|
| 30 Rubber as latex                                                                                       | 100   |
| Sulphur                                                                                                  | 3     |
| Heptaldehyde-aniline condensation product                                                                | 1 1/2 |
| Cocoanut oil soap                                                                                        | 1     |
| 35 Glue                                                                                                  | 1     |
| Nekal                                                                                                    | 1     |
| Anti-oxidant (acetaldehyde-aniline condensation product prepared in a strong acid solution, as emulsion) | 3     |
| 40 Casein                                                                                                | 5     |
| Whiting                                                                                                  | 30    |
| Zinc oxide                                                                                               | 2     |
| Pigment                                                                                                  | 3     |

The Nekal in the above formula is a condensation product of an aromatic hydrocarbon with an aliphatic alcohol in the presence of sulphuric acid. It acts as a preservative and increases the penetrating power of the dispersion. The above formula is merely illustrative, and the ingredients named may be replaced in whole or in part by other suitable ones. For instance, any other accelerator may be used in place of the heptaldehyde-aniline condensation product, but it is preferred in all cases to use an accelerator functioning at a low enough temperature to avoid any possible injury to the fibres by too great or too long heating. Any other suitable anti-oxidant may also be employed, as well as other filling or coloring materials. In making up the latex composition it is diluted with water until the total solid content is approximately 40 per cent.

After the impregnated bat issues from between the rolls 6 and 7, the rubber in it is

coagulated, either by heat or by the use of a coagulant. If heat is used, the bat is passed directly into a heated drying chamber and dried on a traveling belt, on a tentering frame, or in any other suitable manner. If 70 a coagulant is used, the impregnated bat may be sprayed with a weak solution of acid, or instead it may be passed through a bath of the acid. After coagulation by the acid or other coagulant used, the bat may be passed 75 through a series of washing tanks, to remove the coagulant, and then passed into a drying chamber as before, and appears as shown at 8 in Fig. 2. If desired, the bat may be passed through the latex bath a second time and 80 again dried.

From the drying chamber the material is passed through a series of calendar rolls, to bring it to the desired thickness, to give it a uniform surface, and to thoroughly mat the 85 fibres gently together, about as shown at 9 in Fig. 3.

The material is now ready for coating with a rubber compound, and this compound may be conveniently applied by the usual calendering process. However, if desired, the rubber coating may be applied as a dough by the usual form of spreading machine, or instead of a dough of milled rubber, a latex composition prepared for spreading may be 90 used. A suitable rubber compound for coating the material is as follows:

|                                                                 | Parts |
|-----------------------------------------------------------------|-------|
| Crepe rubber                                                    | 26    |
| 35 Softeners (such as paraffin wax, pine tar, Montan wax, etc.) | 4     |
| Ground chrome leather                                           | 15    |
| Formaldehyde-ethylamine condensation product                    | 3/4   |
| Zinc oxide                                                      | 5     |
| Pigment                                                         | 14    |
| Anti-oxidant                                                    | 1     |
| Sulphur                                                         | 3/8   |

The above formula is merely illustrative, and it may be varied in whole or in part to suit conditions. In place of the formaldehyde-ethylamine condensation product, such accelerators as tetramethylthiurammonosulphide, tetramethylthiuramdisulphide, or diphenyl guanidine may be used.

For general purposes, the amount of rubber compound used for coating is controlled by the weight of the felt to start with. In starting with a 16 ounce felt impregnated with 16 ounces of latex compound, it is necessary to coat with 16 ounces of rubber compound, considering the width of the felt 54 inches per linear yard.

If an embossed finish is desired, the rubber coating is next superficially treated with a halogenating material, such as sulphur chloride, in order to set or harden the rubber very slightly in from the surface, so that it will retain the configuration impressed 125 130

upon it by the embossing plates. While the sulphur chloride may be applied in any desired form and by any suitable method, it is preferred to spread a 7½ per cent solution of the sulphur chloride in carbon tetrachloride, as by the spreading operation the reaction can be better controlled. Following the sulphur chloride treatment, the material is then embossed by the use of any common embossing apparatus. Following the embossing step, it may be given a two-tone finish by spreading on the rubber surface a thin rubber cement of a contrasting color to that in the rubber coating compound, so as to more or less fill the indentations formed by the embossing dies. If a plain finish and not an embossed one is desired, the before described sulphur chloride treatment and the embossing may be omitted. The material may also be made up in single colors and embossed. If desired, a coating may be spread or calendered on the inside surface. This inside coating may or may not be embossed.

The embossed or plain sheet is then cured in any suitable manner as in an open heater, and, as before pointed out, it is preferred to use low temperature vulcanizing combinations, both in the impregnating compound and the coating compound, in order that the fibre may not be subjected to an unduly long heat or excessively high temperature.

After vulcanizing the material, the coating is given a finishing treatment with a halogen, which may be a sulphur chloride solution or a bromine solution, but preferably both are used. For instance, the surface of the coating may be first treated with a 7½ per cent solution of sulphur chloride in carbon tetrachloride, and this treatment followed by one with a 2 to 3 per cent solution of bromine in carbon tetrachloride, or instead a single solution is used of the two ingredients in about the same proportions. The successive treatments with sulphur chloride and bromine impart a somewhat hard and glossier surface. However, the combined treatment is a little more convenient, as it involves only a single step. If desired, the vulcanized material may be given a thin coating of shellac before the final surface halogenation, or the vulcanized rubber surface may be halogenated, shellacked, and again halogenated.

It will be seen that by the present invention a sheet material 10 has been produced which is cheap, durable, tough, has a very high resistance to tearing, and uniformity of strength, both crosswise and lengthwise of the fibres, which is waterproof throughout, which has a cut edge resembling that of leather, and which has a surface feeling free from harshness and very similar to that of the ordinary embossed leather used for upholstery, luggage, and other purposes. In addition, the material has great resistance to

temperature changes, it can be made in various thicknesses and degrees of flexibility, and can be readily given any desired color and grain.

Having thus described my invention, what I claim and desire to protect by Letters Patent is:

1. A method of making a leather substitute which comprises impregnating a bat of fibrous sheet material with rubber, applying a coating of rubber to the sheet, superficially treating the coating by halogenation, embossing, vulcanizing, and finally halogenating the finished surface. 75

2. A method of making a leather substitute which comprises forming a sheet bat of mixed vegetable, animal and artificial fibres, impregnating the bat with a water dispersion of rubber, drying, consolidating the bat, applying a coating of rubber, superficially treating the coating with sulphur chloride, embossing, vulcanizing, and halogenating the finished surface. 85

3. A method of making a leather substitute which comprises impregnating a sheet bat of fibres with a water dispersion of rubber, drying consolidating the sheet, applying a coating of rubber, superficially treating the coating with sulphur chloride, embossing, vulcanizing, and forming a finished surface by treatment with bromine. 95

4. A method of making a leather substitute which comprises impregnating a sheet bat of fibres with rubber latex, drying, consolidating the sheet, applying a coating of rubber, superficially treating the coating with sulphur chloride, embossing, vulcanizing, and halogenating the finished surface with bromine and sulphur chloride. 105

5. A method of making a leather substitute which comprises impregnating a sheet bat of fibres with rubber latex, drying, consolidating the sheet, calendering a coating of rubber thereon, superficially treating the coating by the application of sulphur chloride in solution, embossing, vulcanizing, and successively treating the coating with solutions of sulphur chloride and bromine. 115

6. A method of making a leather substitute which comprises impregnating a sheet bat of fibres with rubber latex, drying, consolidating the sheet, applying a coating of rubber, vulcanizing, and finally halogenating the finished surface with bromine and sulphur chloride. 125

7. A method of making a leather substitute which comprises impregnating a sheet bat of fibres with rubber latex, drying, applying a coating of rubber to one surface, superficially treating said coating with sulphur chloride, embossing, applying a coating of rubber on the other surface of the fibrous material, vulcanizing, and halogenating both surfaces with bromine and sulphur chloride. 135

8. A method of making a leather substitute 130

which comprises cross carding fibres into a sheet bat, hardening the bat by moisture and pressure, impregnating the moist bat with a water dispersion of rubber, drying and consolidating the sheet, applying a coating of rubber, vulcanizing, and forming an indurated finished surface by a halogen treatment.

9. A method of making a leather substitute, which comprises cross carding mixed vegetable, animal and artificial fibres into a sheet bat, hardening the bat by moistening and pressure, impregnating the moist bat with rubber latex, drying and consolidating the sheet, applying a coating of rubber, superficially hardening the coating with material comprising a halogen, embossing, vulcanizing, and treating the finished surface with material comprising a halogen.

10. A leather substitute comprising a vulcanized rubber impregnated backing of compacted fibres impregnated with solids deposited from an aqueous rubber dispersion, and a coating of vulcanized rubber having a surfacing of hardened material containing combined bromine.

11. A leather substitute comprising a vulcanized backing of a compressed rubber impregnated bat including vegetable and animal fibres, and an embossed coating of vulcanized rubber having a surfacing of hardened material comprising combined chlorine and bromine.

12. A leather substitute comprising a vulcanized rubber impregnated body of compacted fibres impregnated with solids deposited from an aqueous rubber dispersion, and having on one surface an embossed coating of vulcanized rubber and the other surface a coating of vulcanized rubber, both surfaces superficially halogenated.

Signed at Bristol, county of Bristol, State of Rhode Island, this 19 day of March, 1929.

HAROLD D. RICE.